

Sept. 2, 1941.

E. JUNKER ET AL

2,254,805

PROCESS FOR THE SEPARATION OF METALS

Filed Aug. 22, 1939

Fig. 1



Fig. 2



Fig. 3



Inventors:  
ERICH JUNKER  
By WILLIBALD GEITGEBEL  
Walter O. Tolson  
Attorney.

## UNITED STATES PATENT OFFICE

2,254,805

PROCESS FOR THE SEPARATION OF  
METALSErich Junker, Berlin-Charlottenburg, and Willi-  
bald Leitgeb, Berlin-Wilmersdorf, GermanyApplication August 22, 1939, Serial No. 291,286  
In Germany August 22, 1938

4 Claims. (Cl. 75—63)

The invention relates to the manufacture of metal powder and to the separation of metals by at least partly converting the metals into powder form. It is known that the brittleness of metals increases with increase of temperature, and is extraordinarily high just below the melting point. The range of high brittleness differs according to the various kinds of metals, and lies between the solidifying point and from 5° to 30° C. below that point, as to metals here under consideration. This physical property of metals is used according to the invention to convert simple metals, mixtures of metals or metal alloys into powder.

According to the invention that metal which is to be converted into powder, is submitted to strain by beating, shaking, rolling, grinding or kneading at a temperature below the melting point within the range of high brittleness. Thereby the metal treated breaks down into more or less fine powder, according to the temperature, and the strength of the mechanical forces. Hitherto metal powders have been prepared by breaking up metals without increase of temperature by cutting tools. Also metal foils have been mechanically broken up by stamping, rolling or the like or metals disintegrated by air or steam. Finally molten metals at their melting points, during the occurrence of solidification have been disintegrated to groats by stirring. Over and above these processes the present invention offers the advantage of yielding oxide free metal powder, in a simple manner, in spite of the use of raised temperatures.

A further feature of the invention consists in that single metals are separated from metal mixtures and also metal alloys in such a manner that the metals at least in part are converted into powder. This separating method is applicable to mixtures and alloys of metals in as far as differences of melting point of the single metals or of the alloy components occur. According to the invention the mixture is first heated to a temperature below the melting point but within the temperature range of high brittleness of the lowest melting metal, and at this temperature submitted to a mechanical stressing, e. g. by impact, shaking or beating.

According to the invention the pulverised fraction of the metal is separated in a subsequent operation or, advantageously in the same working process, by sifting or sieving and the remainder again mechanically treated at a higher temperature, but below the melting point and within the range of high brittleness of the metal

5 of the next higher melting point, and the pulverised fraction of the metal again separated. The process can be continued while increasing the temperatures corresponding to the melting points of the metals present until any desired metals are separated from one another.

The process is also applicable to alloys, which consist, e. g. of a crystal component of high melting point and one of low melting point. The 10 alloy is first heated at a temperature under the melting point of the crystal component of the lowest melting point but within the temperature range of high brittleness, and to this temperature submitted to a mechanical stressing, by 15 which the said crystal component is pulverised. Preferably the alloy which is to be separated into its crystal components is previously disintegrated.

The process can for example be applied to the separation of the single metals from mixed turnings or chips of white metal, light metal, red brass, bronze and high melting metals.

*Example 1.*—Separation of a mixture of parts of lead (melting point 327° C.) and aluminum (melting point 658° C.): The metal mixture is heated 20 to approximately 310° C. and then mechanically stressed by shaking, beating or the like. Thereby, the lead entirely disintegrates into powder, whereas the aluminum parts remain unchanged. The powder is simultaneously or subsequently 25 removed by sifting.

*Example 2.*—Separation of a tin component (melting point 232° C.) from a tin-aluminum alloy containing, e. g. 50% tin: Pieces of the alloy are heated to approximately 220° C. and mechanically stressed by shaking, beating or the like. Thereby, the structure of the alloy is broken and a mixture is obtained of coarse aluminum primary crystals and of the eutectic 30 disintegrating to powder which contains all the tin. The powder will be sifted from the aluminum crystals, either simultaneously or subsequently.

*Example 3.*—Separation of a mixture of tin (melting point 232° C.) zinc (melting point 419° C.), aluminum (melting point 658° C.), and copper (melting point 1083° C.). The mixture is heated first to approximately 220° C. and mechanically stressed by beating or the like. Thereby the tin disintegrates into powder which is 45 separated from the other metals through a fine sieve; then, the remainder of the mixture is further heated up to about 400° C. and again mechanically stressed by beating or the like whereby the zinc disintegrates into powder and is removed by sifting. The then-remaining mixture

is heated to about 640° C. and mechanically stressed by beating or the like whereby the aluminum is obtained in powder form and is removed by sifting so that finally the copper remains and all the four metals are separated from each other.

The apparatus for carrying out the pulverisation and separating process according to the invention can be constructed in different manners. We prefer rotating drums with inserted pins, scoops, ribs or the like, in which one of the drums can be stationary or both can rotate. The outer drum can also be formed as a casing. Instead of this a special casing can enclose both drums. The separation of the powder may be brought about advantageously in the same operation as the pulverisation, e. g. if the rotating drum is formed as a sieve drum.

In the drawing are shown diagrammatically three forms of apparatus for carrying out the invention.

Fig. 1 shows a drum, partly broken off, in which a shaft provided with beaters rotates.

Fig. 2 is a diagrammatic cross section through an apparatus in which two concentric drums, provided with beaters, rotate in a single casing.

Fig. 3 shows another form in which several drums rotate besides one another.

The drum *b* according to Fig. 1 is so formed that its parts can be brought to different high temperatures. On feeding in a metal mixture through the feeding hoppers *a* into the end of the drum at the lower temperature (*t*<sub>1</sub>), the metal of the lowest melting point is pulverised by the action of the beating shaft. The powder is led off below through an opening *d* provided with a sieve (compare also Fig. 3). The remaining material passes into a zone of the drum of higher temperature (*t*<sub>2</sub>) in which the metal with the next highest melting point is pulverised and separated and so on.

In Fig. 2 are shown two concentric rotary drums *f*<sub>1</sub>, *f*<sub>2</sub> with beaters which can be formed as sieve drums. Both drums are surrounded by a casing *e*.

In the form according to Fig. 3, three drums *b*<sub>1</sub>, *b*<sub>2</sub>, *b*<sub>3</sub> are arranged alongside one another. The drums of the apparatus may be kept at the same temperature, e. g. when only one metal is to be pulverised. The apparatus can however also be so constructed that the first drum *b*<sub>1</sub> has the lowest temperature, in order to powder the metal of lowest melting point there, and to sieve off the same through the opening *d*<sub>1</sub>, provided with a sieve *s*<sub>1</sub>, while the following drum *b*<sub>2</sub> has a higher temperature, so that the metal of the next highest melting point is separated as a powder and so forth. Drums can also be used at a distance from one another. The metal is then fed from one drum to another by a suitable conveyor.

The process is specially suitable for the manufacture of oxide free aluminium powder, also for working up metal mixtures, in particular for separating the metals of mixed foil waste. In this case after separation of the lower melting metals by fractional pulverisation, finally the metal of highest melting point remaining behind, for example, aluminium, is heated to 400°-550° C., whereby organic components, e. g. paper,

burn or carbonise, preferably with exclusion of air, or with a reduced air supply, and can be separated pneumatically by means of a suction apparatus. In the working up of metal mixtures which are to be pulverised, or which are to be separated by partial pulverisation there can be carried out according to the invention first a mechanical separation in the wet way into specifically heavier and lighter components, e. g. by flotation. In this manner can be separated organic components and impurities, e. g. paper, and moreover a general separation into heavy metals and light metals can be carried out. The thus obtained metallic fractions can then themselves be separated into their components according to the invention in the dry way.

We declare that what we claim is:

1. Process for separating components of metal mixtures comprising heating the mixture up to a temperature below the solidus point but within the temperature range of high brittleness of the lowest melting metal, subjecting the mixture to mechanical stress to reduce the lowest melting metal to powder and separating the powder from the remainder of the mixture.

2. Process for separating components of metal mixtures, comprising heating the mixture up to a temperature below the solidus point but within the temperature range of high brittleness of the lowest melting metal, subjecting the mixture to mechanical stress to reduce the lowest melting metal to powder, separating the powder, heating the remainder of the mixture to a temperature beneath the solidus point of the metal of next highest melting point, again subjecting said remainder of the mixture to mechanical stress, separating the metal powder thereby obtained, from the then remaining portion of the mixture, and repeating the process at constantly increasing temperatures until any desired metals are separated from one another.

3. Process for separating components of alloys comprising heating the alloy up to a temperature below the solidus point but within the temperature range of high brittleness of the lowest melting crystal component, subjecting the said alloy to mechanical stress at this temperature, separating the pulverised alloy component, heating the remainder of the alloy to a temperature below the solidus point of the next highest melting component, subjecting said remainder of the alloy to stress at this temperature, separating the thereby pulverised component from the then remaining alloy components, and repeating the process at constantly increasing temperatures until any desired alloy components have been separated from one another.

4. Process of separating metal mixtures or alloys comprising heating the mixture or alloy up to a temperature below the solidus point but within the temperature range of high brittleness of the lowest melting metal or crystal component present, subjecting the mixture or alloy to mechanical stress to pulverise said lowest melting metal or crystal component, and at the same time separating the non-pulverised metal or alloy residue from the powdered metal or alloy component produced.

ERICH JUNKER.  
WILLIBALD LEITGEBEL.